

April 10, 1945.

C. L. FAUST

2,373,466

METHOD OF ANODICALLY POLISHING ZINC

Filed Nov. 6, 1939



Inventor  
CHARLES L. FAUST

Charles L. Faust Attn.

## UNITED STATES PATENT OFFICE

2,373,466

## METHOD OF ANODICALLY POLISHING ZINC

Charles L. Faust, Columbus, Ohio, assignor to  
 Battelle Memorial Institute, Columbus, Ohio, a  
 corporation of Ohio

Application November 6, 1939, Serial No. 302,954

4 Claims. (Cl. 204—140)

This invention relates to a method of and an electrolyte for anodically polishing zinc and zinc alloys. More particularly the invention relates to an aqueous electrolyte comprising phosphoric acid, chromic acid and water and to the use of such electrolyte in the anodic polishing of zinc.

I have now found that an aqueous electrolyte comprising phosphoric acid, chromic acid and water, as the essential ingredients, can be satisfactorily used in the anodic polishing of zinc, zinc base dies casting alloys, zinc alloys commonly used in extrusion processes and, in general, any zinc alloy containing more than 50% of zinc. If the relative proportions of the three ingredients of the bath be kept within certain limits, which I have determined, very satisfactory polishes can be produced in the case of zinc, while at the same time obtaining surfaces having relatively superior characteristics to those prepared by mechanical polishing or buffing operations. Best results are obtained on zinc itself, or on alloys of zinc containing over 90% of zinc.

It is therefore an important object of my invention to provide an electrolyte containing phosphoric acid, chromic acid and water within certain limits as to their relative proportions, for use in the anodic polishing of zinc and zinc alloys to impart thereto a highly lustrous surface.

It is a further important object of this invention to provide a method of anodically polishing zinc and zinc alloys using an electrolyte of novel composition that is operative throughout a wide range of anode current densities and temperatures.

Other and further important objects of this invention will become apparent from the disclosures in the specification and the accompanying drawing.

This invention (in its preferred form) is illustrated in the drawing and hereinafter more fully described.

On the drawing the figure represents a triaxial diagram showing the relative proportions of phosphoric acid, chromic acid and water in compositions of electrolyte coming within the scope of my invention.

In the accompanying diagram, the respective sides of the triangle indicate the percentages of phosphoric acid ( $H_3PO_4$ ), of water ( $H_2O$ ), and of chromic acid ( $CrO_3$ ), from 0 to 100%. On the basis of experimental data, I have determined the relative proportions of phosphoric acid, chromic acid and water that give compositions of electrolyte that are operative for the anodic polishing of zinc. The area representing opera-

tive compositions of electrolyte is defined on the accompanying diagram by the solid lines AB, BC, CD, and DA. Within the area so defined, any composition selected will be found to be operative in the method hereinafter described for the anodic polishing of zinc.

In order to get the best polishing results, however, I have found that the range of proportions of phosphoric acid, chromic acid and water should be kept within somewhat narrower limits and these narrower limits are represented on the accompanying diagram by the area defined by the lines AB, BE, dot and dash lines EF, and FA. The preferred compositions of electrolyte, with respect to the relative proportions of phosphoric acid, chromic acid and water, lie within this second lesser area, which is wholly enclosed within the broader area first defined.

The reading of a triaxial diagram such as the accompanying one is well understood, but the following will be given for purposes of illustration. The point on the diagram represented by the letter A, for instance, indicates a composition comprising a small but significant proportion, say 20 0.1% of phosphoric acid, 65% of chromic acid and the balance, somewhat less than 35%, water; the point indicated by the reference letter B a composition comprising 85% of phosphoric acid, say about 0.1% of chromic acid and the balance, somewhat less than 15%, water; the point indicated by the reference letter C a composition comprising 32% phosphoric acid, say about 0.1% of chromic acid and the balance somewhat less than 68%, water; and the point represented by the reference letter D a composition comprising say about 0.1% of phosphoric acid, 49% of chromic acid and the balance, somewhat less than 51%, water.

It will be seen that the maximum phosphoric acid content is 85% and the minimum about 0.1%, the maximum chromic acid content 65% and the minimum about 0.1%; the maximum water content about 68% and the minimum 13%. The preferred composition limits are from 0.1 to 85% phosphoric acid, from 0.1 to 65%  $CrO_3$  and from 13 to 56% water. The relative proportions of phosphoric acid, chromic acid and water, however, are inter-dependent, so that instead of selecting a bath composition having percentages within the maximum and minimum ranges for the three ingredients, the composition of electrolyte should be selected by reference to the triaxial diagram and a point selected within the preferred area if best results are to be obtained.

While the accompanying triaxial diagram indi-

cates relative percentages of phosphoric acid, chromic acid and water in a system consisting of only these three components, suitable bath compositions of these three components may nevertheless contain other ingredients, such as acids other than phosphoric and chromic acids, and/or salts. From the diagram, however, the relative proportions that phosphoric acid, chromic acid and water should bear to each other may be determined for operative and preferred ranges of composition, regardless of what other non-essential ingredients may be present in the bath.

Thus, for instance, in making up an electrolyte for the anodic polishing of zinc, one might select the point X on the triaxial diagram as being a bath of preferred composition. The composition represented by the point X would be 60% phosphoric acid, 10% chromic acid and 30% water. During the continued use of such a bath in the electropolishing of zinc, the bath composition would necessarily change, owing to the anodic dissolution into the bath of zinc. There might also be some change in the water content, such as an increase due to absorption by the bath of moisture from the air, or a decrease due to evaporation of water from the bath, to decomposition of water by electrolytic action, or to loss of water from the bath by entrainment thereof in gases given off from the bath.

Notwithstanding such changes in its composition as may occur during continued use, if the relative percentages of phosphoric acid, chromic acid and water, expressed as percentages by weight of the total weight of only these three ingredients in the bath composition, remain within the area defined by the lines AB, BE, EF and FA, the bath will continue to operate satisfactorily. Even if the bath composition be so altered during continued operation that it falls within the less preferred area defined by the lines FE, EC, CD and DF, on the accompanying diagram, the bath will continue to function, although not so satisfactorily.

Consequently, where the relative percentages of phosphoric acid, chromic acid and water in a given bath composition lie within either the preferred or less preferred areas defined on the triaxial diagram, such bath composition is intended to come within the scope of my invention, even though it may contain other acids than phosphoric and chromic and even though it may contain a substantial quantity of metallic salts. Instead of chromic acid, soluble chromates and bichromates may be substituted therefor and are to be considered the equivalent of chromic acid on a stoichiometric basis. The term "chromic acid equivalent," as used in this specification and in the claims, is therefore intended to include chromic acid itself ( $\text{CrO}_3$ ) and stoichiometrically equivalent weights of soluble chromates and bichromates.

Similarly, in place of orthophosphoric acid, other phosphoric acids, such as meta- and pyrophosphoric acids, may be used and are to be considered as included within the term "phosphoric acid."

In the method of anodically polishing zinc, using a bath of a composition indicated as suitable by reference to the accompanying triaxial diagram, the zinc, or an article having a surface of zinc, is made the anode in a bath of the selected composition and an electric current is passed therethrough of sufficient density and for a sufficient length of time to produce the desired high degree of luster, or polish, on the surface of the

zinc. By employing an electrolyte having a composition within the preferred area defined on the accompanying triaxial diagram, a highly lustrous, mirror-like surface can be readily obtained. The highly lustrous surface obtainable by my method, using an electrolyte of preferred composition, is an important feature of my invention and one that sharply distinguishes it from prior art finishes produced in the electrolytic cleaning of metals.

The formation of highly polished and lustrous surfaces is undoubtedly associated with the presence of a polarizing film over the surface of the metal during the process of anodic dissolution. The nature of this film is such that selective attack on the various phases present in the zinc, or zinc alloy, is minimized. Anodic dissolution apparently takes place at a relatively high rate and at a high anodic polarization value, with the result that the anodic dissolution of the metal acts to level the crystal surfaces thereof and to produce a mirror-like finish. These conditions do not prevail in the simple electrolytic cleaning treatment known to the prior art.

In order to obtain the best results in a reasonable length of time, it is preferable to use controlled voltages of 1 to 15 volts, at which the current density will suitably adjust itself to a value within the range of 3 to 150 amperes per sq. ft. It will be found that higher densities can be used in baths of high phosphoric-chromic acid ratio, for example up to 500 amperes per sq. ft., for which the voltage will be from 20 to 30 volts. Higher current densities may be employed but are necessarily more costly because of the higher voltages required and the consequent higher cost of electrical energy. The length of time to effect the desired results depends upon the magnitude of the current densities employed and to some extent upon the particular characteristics of the zinc, or zinc alloy, to be polished, and also upon the character of the surface of the zinc initially. Rough surfaces, of course, require a longer time to polish than relatively smooth ones.

With any of the compositions of electrolyte lying within the preferred area defined by the lines AB, BE, EF and FA, on the accompanying triaxial diagram, excellent polishes are obtained upon zinc, when the zinc, or a zinc coated article, is made the anode therein at a voltage of 3 volts and the treatment is carried out for a period of 1½ to 12 minutes, employing a bath temperature lying within the range of 60 to 100° F. The current density will adjust itself to within the range of 4 to 100 amps./sq. ft. depending upon the  $\text{H}_3\text{PO}_4\text{-CrO}_3$  ratio in the bath. In general the temperature should not exceed 125° F.

From the foregoing description of my invention, it will be apparent that I have provided a novel composition of electrolyte and a method whereby the same may be used to produce highly lustrous polishes on zinc and zinc alloys high in zinc content. My electrolyte and method avoid the disadvantages of the old methods of mechanical polishing and enable the production of zinc, and alloys of zinc, such as zinc base die castings, extruded zinc articles and the like, with surfaces that are free from mechanical strain, dragging and "piling," and which are superior to those obtainable by mechanical polishing methods.

It will, of course, be understood that various details of the process may be varied through a wide range without departing from the principles of this invention and it is, therefore, not the purpose to limit the patent granted hereon other-

wise than necessitated by the scope of the appended claims.

I claim as my invention:

1. The method of anodically polishing an article having a surface of metal selected from the group consisting of zinc and alloys thereof containing more than 90% zinc, which comprises making the article the anode in an aqueous solution comprising essentially  $H_3PO_4$ ,  $CrO_3$ , and water, the percentage proportions by weight of said three solution ingredients lying within the area defined in the accompanying diagram by the line AB, the straight line BC, the line CD and the straight line DA, and at a temperature not in excess of 125° F., passing an electric current therethrough of sufficient density and for a sufficient duration of time to effect a polish on said surface.

2. The method of anodically polishing an article having a surface of metal selected from the group consisting of zinc and alloys thereof containing more than 90% zinc, which comprises making the article the anode in an aqueous solution comprising essentially  $H_3PO_4$ ,  $CrO_3$ , and water, the percentage proportions by weight of said three solution ingredients lying within the area defined on the accompanying diagram by the line AB, the straight line BE, the line EF and the straight line FA, and at a temperature not in excess of 125° F., passing an electric current

15 30

therethrough of sufficient density and for a sufficient duration of time to effect a polish on said surface.

3. The method of anodically polishing an article having a surface of metal selected from the group consisting of zinc and alloys thereof containing more than 90% zinc, which comprises making the article the anode in an aqueous solution comprising essentially  $H_3PO_4$ ,  $CrO_3$ , and water, the percentage proportions by weight of said three solution ingredients lying within the area defined on the accompanying diagram by the line AB, the straight line BE, the line EF and the straight line FA, and passing an electric current therethrough at a voltage of from 1 to 15 volts at a solution temperature of from 60° to 100° F.

4. The method of anodically polishing an article having a surface of metal selected from the group consisting of zinc and alloys thereof containing more than 90% zinc, which comprises making the article the anode in an aqueous solution comprising essentially  $H_3PO_4$ ,  $CrO_3$ , and water, the percentage proportions by weight of said three solution ingredients lying within the area defined on the accompanying diagram by the line AB, the straight line BC, the line CD and the straight line DA, and passing an electric current therethrough at a voltage of from 1 to 15 volts at a solution temperature of from 60° to 100° F.

CHARLES L. FAUST.